

June 5, 1928.

1,672,402

E. R. ARMSTRONG

## PLATING APPARATUS AND PRODUCT THEREOF

Filed Oct. 14, 1924

2 Sheets-Sheet 1

Fig. 1



Fig. 2

Inventor

E.R. Armstrong,  
By his attorney *J.P. Sguar*.

June 5, 1928.

1,672,402

E. R. ARMSTRONG

## PLATING APPARATUS AND PRODUCT THEREOF

Filed Oct. 14, 1924

2 Sheets-Sheet 2



Fig. 4



Fig. 5



### Electrolytically deposited metal belt (nickel)

46<sup>a</sup> Fig. 10



Fig. 9



Fig. 8

Inventor  
E.R. Armstrong,

Attorney  
*F. R. Squair.*

## UNITED STATES PATENT OFFICE.

EDWARD R. ARMSTRONG, OF HOLLYOAK, DELAWARE, ASSIGNOR TO E. I. DU PONT DE NEMOURS & COMPANY, OF WILMINGTON, DELAWARE, A CORPORATION OF DELAWARE.

## PLATING APPARATUS AND PRODUCT THEREOF.

Application filed October 14, 1924. Serial No. 743,589.

This invention relates to apparatus for the production of continuous metallic strips by the electrolytic deposition of the metal, and to the product thereof, and, in particular it 5 has to do with apparatus comprising a continuously driven cathode from which the deposited metal is continuously stripped in an "endless" band, that is, a band of indefinite length. Previous attempts to produce such 10 a band have been unsuccessful, there not having been produced a band satisfactorily free from pitting and other imperfections; this being due, I have found, to failure to maintain the electrodes in proper condition, or 15 to maintain the solution in sufficient agitation and free from impurities, or take various other precautions. A further difficulty has been that it was not possible to produce continuous strips of a thickness, width and 20 strength, adapting them for use as continuous belts of such long span, width and stability as to make them possible for use as casting belts on which to deposit solutions in the making of continuous strips of cellulose-ester materials, for example, nitrocellulose films, by casting and evaporation of 25 solvents. It is an object of this invention to provide an apparatus of the character indicated in which the various prior difficulties 30 are overcome and with which strips suitable for use as belts in the field just mentioned can be made. It is also an object to provide such a strip. To these ends, and also to improve generally upon devices of the character 35 indicated, the invention consists in the various matters hereinafter described and claimed. For definiteness, the invention is here described with more particular reference to the making of nickel strips or belts, 40 and to the illustrated apparatus, but it will be understood that the invention is not confined to the making of strips of a particular metal nor to the illustrated embodiment.

In the accompanying drawings:

45 Figure 1 is a side elevation, partially in section, of an apparatus of the present invention as a whole;

50 Figure 2 is a vertical longitudinal sectional view of the electrolytic plating device, but with the cathode drum and its driving means, and certain closely related parts unsectioned and in elevation;

55 Figure 3 is a plan view of the plating device, and certain closely related parts;

Figure 4 is a fragmental face elevation of 55 the plating drum, or cathode, sectioned in part;

Figure 5 is a fragmental side view of the rim of the plating drum;

Figure 6 is a plan view of the clearing or 60 bubble-removing device;

Figure 7 is a plan view of the rack device for operating the bubble-removing device, its side arms being broken out to save space, and it being shown lower-face-up, the better 65 to show the racks;

Figure 8 is a plan view of the roller for confining the departing strip.

Figure 9 is a top view, with the casing sectioned, of the reduction gear for driving the 70 cathode; and

Figure 10 is a conventional illustration of the product.

Referring now to the drawings, and more particularly to Figure 1, the assembly 75 comprises a plating device, designated generally as 1 and comprising a tank 2 for electrolyte solution, an anode 3 and a cathode 4, a storage tank 5, a filter tank 6 with filters 6<sup>a</sup> desirably of filter duck, a hard rubber pump 7 drawing from the storage tank, pipe connections 8 from the storage tank to the filter tank, pipe connections 9, 9, from the filter tank to the tank of the plating device, pipe connections 10 from the plating tank to the 85 storage tank, an overflow pipe 11, and driving means designated generally as 12 for the cathode and other driven parts. The cathode is in the character of a drum having a metallic peripheral plating surface or face, and 90 is partially immersed in the electrolyte in the tank 2. The various tanks may be of wood and the piping of rubber-lined hose with hard rubber connection. In operation, as the driving means slowly rotates the 95 cathode 4 (anti-clockwise in the drawing) the metal from the anode is deposited (by way of the solution) on the periphery of the cathode and is stripped off in an endless band B. Meanwhile the solution is continuously in agitation and movement and is being continuously cleaned, it being circulated from the tank 2 around the circuit 2—10—5—7—8—6—9, 9,—2 and being filtered in the tank 6; any excess in the tank 6 overflows by the pipe 11 to storage. The tank 2 is desirably kept closed at the top so far as 100 feasible to prevent the hot vapors from the

tank reaching the cathode surface and strip.

Now to describe in detail certain features of the plating device:—The tank 2 supports the anode 3 and cathode 4, the latter being journaled by the bearings 14, 14 upon the tank for rotation upon its axis. The anode 3 comprises, in accordance with the invention, a pair of spaced partitions 15 and 16

reaching across and supported by the tank. 5 journalled by the bearings 14, 14 upon the tank for rotation upon its axis. The anode 3 comprises, in accordance with the invention, a pair of spaced partitions 15 and 16 reaching across and supported by the tank.

10 These partitions are of sheet material of a character to properly withstand the action of the solution, and to not be plated upon, as phenolic resin (bakelite) or cellulose ester plastic (pyralin) and are each perforated,

15 as at 17, for passage of the solution. These partitions provide between them a confining space 18 within which is received the anode proper. This consists of pellets 19 of the metal to be deposited, for example, nickel.

20 With this construction the anode can at any time be conveniently renewed, it merely being necessary to load in pellets at the open ends 18<sup>a</sup>, 18<sup>a</sup> of the space 18 as occasion requires. In this way I provide for the replen-

25 ishing at will of the metal being plated out, without interruption of the operation, thus readily permitting the continuous operation which I desire. Desirably the upper partition conforms to the curve of the periphery

30 of the cathode but is somewhat spaced therefrom. Preferably the lower partition 16 is given a V-shape with each half approximating

35 at the angle of repose of the pellets thus to ensure that the hidden parts of the space

35 18 shall always contain pellets, provided the upper portions, which are observable at 18<sup>a</sup>, 18<sup>a</sup>, contain pellets, all danger of there being a concealed "empty space" being eliminated.

40 The positive lead (see Figure 2) may desirably be connected with a bus bar 20 having projections 21.

As before stated the cathode 4 is in the character of a rotating drum. As here shown it comprises (see Figure 4) an iron (steel) rim 22 fast supported upon the shaft

45 23 (Figure 3) by the metal arms 24. At each end the central opening of the cathode is closed solution tight with a wooden head

50 25. Carried upon each head 25 is a peripheral upstanding rim 26, extending throughout the length of the periphery, which

55 serves to confine the plating. These rims are of some material, for example, wood, bakelite or pyralin, unaffected by the bath and upon which the metal will not plate.

For convenience in construction they are each in several arc-shaped pieces (Figure 5) and in order to ensure that there shall be no creeping of the solution along the line

60 of the joint 27, a pin 28 is tightly driven into the joint which seals the same against creeping of the solution therealong. In further accordance with the invention the rims are provided with a series of closely adja-

65 cent arc-shaped protectors 29, closely over-

hanging the plating surface but sufficiently distant therefrom to permit a deposition of the desired thickness. These protectors extend throughout the circumference of the rim except for such length as it is desirable 70 to provide for the convenient stripping off of the band B, and to provide this length the protectors are received with a push fit in sockets 30 in the rim so that as the drum turns (the movement is slow) they can in 75 turn be removed to provide the said "length" and then replaced when the need for the "length" at that particular portion of the rim has passed. These protectors are of a material unaffected by the solution and upon 80 which the metal will not plate and are desirably of bakelite or pyralin. They serve to prevent "treeing" of the deposit at the corner 31 between the plating surface and rim. The steel surface of the cathode is desirably plated with copper and then nickel, the same being polished to that degree necessary to give the finish desired on the deposited strip. The negative lead is conveniently connected with brushes-and-slip-ring 32 (Figure 3) contacting the shaft 23 which in turn is in connection with the rim by way of the arms 24. The drive of the cathode is by the heretofore mentioned mechanism 12 to be described in detail herein- 85 after.

A clearer or bubble remover 33 is provided. Referring more particularly to Figures 2 and 6, the same comprises the brush bristles 34 held in the hard rubber back or cross bar 35 and extending from side to side across the plating surface and in contact therewith. Desirably the brush is oscillatable about the axis of the cathode to travel over substantially the entire immersed surface thereof, the space 36 between the cathode and the anode partition 15 permitting this. To provide for this oscillation, as here shown the brush is carried between arms 37, 37 (say, of wood) each fast at its end to a gear wheel 38, loose upon the shaft 23 of the cathode. A rack frame 39 (Figure 7) presents two racks 40, 40 each in mesh with a respective gear 38. The frame is driven (Figure 3) by the pitman-and-crank 41 from the shaft 42 of the driving mechanism 12. With this arrangement the deposit is kept free of hydrogen bubbles and any suspended impurities and a proper deposit without pits or other imperfections is ensured.

A guide roller 43, preferably of steel covered rubber, for the departing finished strip is provided, see Figures 2 and 8. As here shown it extends crosswise the casting surface, parallel and adjacent thereto, being carried by arms 44, 44<sup>a</sup> the one, 44, carried loose upon the shaft 23, and the other fixed upon the gear-box 12<sup>b</sup> of the driving mechanism, the gear-box oscillating if the cathode is to oscillate, and being stationary if

the cathode is not to oscillate, as hereafter described in connection with the drive. The gear-box, and hence the roller, may be held against oscillation by a member 45 (Figure 3) secured to the tank and the gear-box. This roller ensures that the deposited strip will not pre-depart from the casting surface. Conveniently the roller is supported in bearings 46, 46 carried by studs 46<sup>a</sup>, 46<sup>b</sup> slidably secured in a cross-piece 47, tension springs 48, adjustable at 49 in the well-understood manner, serving to urge the roller into contact with the band B while permitting yielding on account of irregularities or the like.

At each end of the roller 43 there is carried to rotate therewith an edged cutting or marking disc 43<sup>a</sup> which discs serve to mark off longitudinally of the band B a straight strip of uniform width.

Desirably, structure is provided for the convenient buffing and cleaning of the plating surface. Thus, as here illustrated (Figure 1) a pair of swing arms 50, are borne, one at each side of the tank 2, in bearings 51, which arms are of a length to bring their bearings 52 into register with the shaft 23 when they are swung to overlie the tank. The bearings 52 are closable about the shaft 23 and when they have been so closed the arms, carrying the cathode, are swung back to place the shaft 23 in the pillow blocks 53, in which location the cathode may be dressed or otherwise treated as desired (as by the polisher P).

The tank 2, at those points where the solution supply pipes 9, 9 discharge into the same is shown as provided with a weir-like foam trap or trough comprising the receptacle 54, baffle walls 55 and 56 and weir wall 57. With this construction the inflowing solution must pass the baffles and flow over the wall 57 before entering the tank 2 proper, wherefore any foam is prevented from entering the tank; and also the flow is equalized.

Next to describe the driving mechanism heretofore designated generally as 12:—This mechanism comprises (Figures 1, 2 and 9), in its portion which is immediately related to the cathode, devices whereby the cathode may be given merely a simple rotation, or may be given a rotation combined with oscillation, the cathode oscillating forward and back and at the same time slowly advancing.

Carried loose upon the shaft of the cathode is the reduction-gear-box 12<sup>b</sup> containing the reduction train 58—60, 61—62, 63—64, 65, of which the driving member is ratchet wheel 58 and the final driven member is the shaft 23 to which the gear 65 is keyed. Swinging loose upon the shaft 66, to which member 58 and gear 60 are keyed, is a struck arm 67 which carries the spring pressed feeder pawl 68 meshing the ratchet wheel 58 to advance the same (clockwise) when the arm 67 swings to the left (in Figure 2). A spring pressed holder pawl 69 is carried on the box 12<sup>b</sup> to hold the wheel 58 upon retreat of the arm 67. A pitman-and-crank 70 drive 70 drives the arm 67 from the driving shaft 42, the end of the rod 71 of the pitman-and-crank being pivotably supported by a link 72 loose upon the shaft 23, and having adjacent its so-pivoted end an adjustable striker cam 73 which at each stroke strikes and swings the arm 67, thus advancing the cathode. When the gear-box 12<sup>b</sup> is held against oscillation, as by the member 45 connecting the gear-box 12<sup>b</sup> and tank, the motion of the cathode is, evidently, a simple step-by-step rotation. In order, if desired, to combine with this rotation, oscillation of the cathode, it is but necessary to remove the member 45 and bolt the link 72 to the box 12<sup>b</sup> as by the clamp bolt 74 (see Figure 2 as distinguished from Figure 1). With this change, the rod 71 not only moves the ratchet 58 but also oscillates the gear-box 12<sup>b</sup>. The various meshing or connected units being mounted in the gear-box and the wheel 65 being keyed to the shaft 23, the cathode will be oscillated while at the same time the step-by-step rotation will continue. It will be understood that the sizes and location of the parts are such that even when the gear-box 12<sup>b</sup> is being oscillated the striker cam overtakes and properly moves the struck arm 67. Desirably the oscillation may be about one hundred degrees. Evidently the roller 43 oscillates with the cathode, its arm 44<sup>a</sup> being fast connected with the gear-box. The shaft 42 is shown as driven by the motor 75 through the reduction gear 76. The pump 7 may be driven in timed relation with the other units as by the motor 77, or from the motor 75.

I am aware that it has been previously proposed to electrolytically deposit metal upon a travelling cathode and remove the deposit but, so far as is known, prior devices have not been capable of producing deposits of such quality, stability and thickness as would permit of the production of strips usable as metal belts for film casting, the excessive thinness (lack of strength) of the deposits and their poor quality, as regards porosity, foreign matter and so on, absolutely precluding them from such use. With the present device, it having provisions as described above for removing bubbles, for constant flow of solution, ready renewal of the anode without interruption of the operation, elimination of foam, and so on, I am able to produce heavy, strong, high quality strips well capable of use for long span belts. These belts find use in, and indeed render possible, the casting of cellulose ester solutions into continuous strips, the belt of present production serving

as a continuous traveling casting surface, as described in my United States application Serial Number 743,590, filed October 14, 1924 entitled Machine for casting composition sheets and method of making such sheets.

As an example of the production of such a strip I give the following, the strip produced being about  $2\frac{1}{2}$  feet wide, of the great

10 thickness, as compared to previous abortive efforts, of .035 inch and of a length of substantially 120 feet, which could have been indefinitely increased had it been desirable.

15 Diameter of cathode, 4 feet; width of cathode,  $2\frac{1}{2}$  feet; peripheral speed of cathode, 4.25 inches per hour; bath,  $28^{\circ}$  Bé. solution of nickel sulfate, to which was added 4 cc. of 100% acetic acid per liter and a daily addition of about 1.6 cc. of 7% hydro-

20 gen peroxide per liter; solution in system about 575 gallons, and plating tank maintained substantially full of solution; rate of flow through circuit about 40 gallons per minute; temperature of bath,  $120-130^{\circ}$  F.

25 which was automatically maintained by the electrical energy used in plating; current density, 57 amperes per square foot giving a total current of 720 amperes at 9-10 volts; hydrogen ion concentration, very low when

30 starting with a new bath and anode material but as the solution was purified by the peroxide and filters, and as the anode was worked in, the hydrogen ion concentration rose from less than 3.0, to 3.7 at the end of

35 the run; bubble brush oscillation period 10.6 per minute, the wheel surface being advanced .00667 inch for each stroke; strip produced per day  $8\frac{1}{2}$  feet; time for producing total strip 14 days. To make the strip

40 easily removable from the cathode, after emergence from the bath, the cathode surface was treated with a 0.5% selenious acid solution, applied with a felt wiper, between the points of stripping and of entering the

45 bath again. During the run the anode was renewed as required by supplying additional nickel pellets between the confining sheets. With the present apparatus strips from .01 to .05 in. thick and upward can be readily

50 produced, in widths as great as desired, previous possible strip deposits having at the most a thickness of .0025 in.—a thickness entirely too small for belts for present desired film-casting-belt uses. The present

55 strip has a tensile strength of about seventy to eighty thousand pounds per square inch. Upon completion of a strip of the desired length it may be smoothed and polished in the usual ways of the art. In joining the

60 ends of the strip to make a closed belt, the ends may be closed, dove-tailed crosswise of the strip, and the joint silver brazed, a riveted-on backing strip being used if desired, and the joint smoothed and polished.

I claim:

1. In a plating device, an electrode presenting a plating surface and an upstanding longitudinally extending edge-guarding projection of non-plateable material, said projection comprising a plurality of abutting sections, and means fitted liquid tight between said sections thereby to prevent travel of the plating solution along the line of abutment.

2. In a plating machine having a traveling plating surface and provisions for removal of the deposited metal therefrom in strip form, an upstanding guarding projection extending longitudinally of the plating surface, and treeing-preventing means overhanging said surface from said projection, such means comprising a plurality of sections removably mounted along said projection whereby selected ones of said sections may be removed to permit unhindered removal of the strip deposit from the plating surface.

3. In a continuous plating machine, in combination, a bath tank, a substantially cylindrical cathode mounted with its axis substantially parallel to the surface of the bath and with a portion of its peripheral plating surface immersed in the bath and the remainder exterior of the bath, whereby upon rotation of the cathode the plating surface travels into and out of the bath, an upstanding guarding rim extending throughout each edge of the plating surface, and a treeing guard extending along each rim and overhanging the plating surface, such treeing guard comprising a plurality of adjacent sections removably received in the rim, whereby said sections may be removed from the rim to permit unhindered stripping of the deposit from the plating surface, and replaced when each selected portion of the surface has passed the stripping point.

4. In a continuous plating device, in combination, a bath tank, a substantially cylindrical cathode mounted on said tank to rotate partially immersed therein, and an anode comprising an upper and a lower spaced perforated partition approximately conforming to the curve of said cathode, and a plurality of individual elements of anode metal received in the space between said partitions and constituting the anode proper, said space having an entrance providing for the loading in of said anode elements on occasion.

5. In a plating device, in combination, a bath tank, electrodes therein, means for supplying solution to said tank, such means comprising a solution discharge device discharging into said tank, and means in co-operative relation with said discharge device and tank for equalizing the flow into the tank.

6. In a plating device, in combination, a bath tank, electrodes therein, means for sup-

plying solution to said tank, such means comprising a solution discharge device discharging into said tank, and a weir-box device directly receiving the entering solution and discharging the same to the tank.

5 7. In a plating device, in combination, a bath tank, electrodes therein, means for supplying solution to said tank, such means comprising a solution discharge device discharging into said tank, and a combined foam-baffle-and-weir-box device directly receiving the entering solution and discharging the same to the tank.

10 8. In a plating machine, in combination, a rotatable electrode, and means for rotating said electrode and meanwhile oscillating the same about its axis of rotation.

9. In a plating machine, in combination, a rotatable electrode, means for rotating said electrode, and optionally operative means, cooperative with the rotating means for oscillating the electrode about its axis of rotation.

15 10. In a plating machine, in combination, a rotatable electrode, and means for rotating said electrode and meanwhile oscillating the same, such means comprising a reduction-gearing casing, a reduction gearing therein, and connected with said electrode to rotate the same, means for driving the reduction gearing, and provisions whereby said driv-

ing means may oscillate the reduction-gearing casing thereby to oscillate the electrode during driving of said reduction gearing and rotation of said electrode.

35

11. In an assembly for the continuous electrolytic production of metallic strips, in combination, a plating bath tank, a substantially cylindrical cathode rotatably mounted with respect to said tank to have its peripheral plating surface descend into and emerge from the bath upon rotation, means associated with said plating surface for confining the deposit, an anode in said tank and approximately conforming to the curve of 45 said cathode and somewhat spaced therefrom, driven cathode clearing means oscillatable in said space, a solution circuit for discharge of solution into said tank and withdrawal of it therefrom, driven means 50 for causing said circulation, means associated with said tank and solution for preventing foam in said tank, and continuously operating driving means for driving said cathode, for driving said circulation device to cause solution to be cleared of foam by said foam preventing device and to circulate through said tank, and for driving said cathode clearing device, all in timed relation.

55 In testimony whereof I affix my signature.

EDWARD R. ARMSTRONG.